

October 22, 1966

## UNITED STATES PATENT OFFICE

2,409,687

SULFUR AND METAL CONTAINING  
COMPOUND

Dilworth T. Rogers, Teaneck, and John G. McNab, Cranford, N. J., assignors to Standard Oil Development Company, a corporation of Delaware

No Drawing. Application August 1, 1944,  
Serial No. 547,640

2 Claims. (Cl. 260—125)

1

This invention relates to a novel type of organic compound containing sulfur and a metal.

This is a continuation-in-part of our co-pending application Serial No. 486,428, filed May 10, 1943.

It is known that the addition of certain types of metal organic compounds to lubricating oils improves various properties thereof, such as their oiliness characteristics and their detergent action in engines, particularly manifested in the maintenance of a clean engine condition during operation. Various metal compounds which have been used for such purposes include the metal derivatives of such organic compounds as fatty acids, naphthenic acids, sulfonic acids, alcohols, phenols and ketones. However, these various metal compounds generally have the disadvantage of tending to corrode alloy bearings, such as those of cadmium-silver and copper-lead, now so widely used in automotive engines, and this is especially true in engines which operate at relatively high speeds and high temperatures. It is an object of the present invention to provide a new class of addition agents for oils which are to be used as crankcase lubricants for internal combustion engines and which exhibit the desirable properties of promoting general engine cleanliness, improving oil film strength, reducing ring sticking, piston skirt varnish formation and the like, and which not only do not exhibit the corrosion promoting tendencies characteristic of the above metal compounds, but also inhibit the corrosiveness of oils to which they are added.

The new class of products which have now been found to be highly satisfactory as addition agents are the products obtained by the reaction of elemental sulfur with metal salts of hydroxy and mercapto substituted aromatic sulfides. When these compounds are to be used as additives for mineral oils, they should contain as a substituent in the aromatic nucleus at least one alkyl group, the total number of carbon atoms in such groups being at least five. It has been found that such products are usually satisfactory in inhibiting bearing corrosion and in being adaptable to use with a wide variety of petroleum lubricating oil base stocks. The reaction for the preparation of the additives may generally be brought about in a solution of lubricating oil or other petroleum oil, whereby concentrates may be prepared which may be conveniently stored or shipped and added to lubricating oils when required.

The new sulfur containing compositions herein described are also useful as antioxidants for other purposes when incorporated in organic materials

2

other than lubricating oils, as will be more fully explained hereinafter, and in some cases it may not be necessary to have alkyl groups present in order to impart sufficient solubility. The invention also includes the reaction products of sulfur with compounds analogous to the salts of phenol sulfides and thiophenol sulfides, but containing selenium and tellurium in place of oxygen or sulfur, and with compounds in which aromatic nuclei other than benzene nuclei are present.

In the aforementioned co-pending application Serial Number 486,428 we have described the preparation of reaction products of elemental sulfur with metal phenates and the use of such products in lubricating oil compositions. It was there shown that the sulfur atoms were probably linked directly to the metal atoms in the molecules of the reaction product. It is believed that the same type of reaction occurs when metal salts of phenol sulfides and the like are treated with sulfur, giving compounds in which the sulfur atoms are thought to be attached directly to the metal atom.

Some of the more preferred products to be used in accordance with the present invention are those obtained by reaction of sulfur with the following compounds:

Barium tert.-octyl phenol sulfide  
Barium di-tert.-amyl phenol sulfide  
Calcium isohexadecyl phenol sulfide  
Tin wax-alkylated salicylic acid sulfide  
Magnesium tert.-amyl phenol sulfide

The invention includes the reaction products of sulfur with not only the normal metal salts of phenol sulfides, thiophenol sulfides and the like, but the basic metal salts as well. In a normal phenol sulfide salt of a divalent metal the ratio of metal to phenol sulfide is 1:1 as in the following formula:



In a basic salt the ratio of metal to phenol sulfide may be 2:1 or even 3:1. In the case of a 2:1 ratio the formula may, for example, be



## 3

In the case of a 1.5:1 ratio the formula may be



In the case of a 3:1 ratio the formula may be



Intermediate ratios of metal to phenol sulfide, such as 1.8:1 or 2.3:1, may occur in which mixtures of the above types of basic compounds are obtained. These basic salts are formed, for example, by reacting phenol sulfides with more than the amount of metallic oxide or hydroxide necessary to form the normal salts. Reaction products of sulfur with basic metal salts of alkyl phenol sulfides are particularly useful in extreme pressure lubricants. These products are also especially advantageous for imparting color stability to lubricants.

The new class of addition agents employed in accordance with the present invention may be defined in its broadest scope as the reaction products of elemental sulfur with a metal salt of a compound having the formula



in which Ar is an aromatic nucleus and may, for illustration, be a benzene nucleus, or it may consist of a plurality of rings, as in biphenyl, or it may be a condensed nucleus, exemplified by naphthalene, anthracene and the like. R in the formula is hydrogen or at least one organic group and is preferably an alkyl group. X in the formula is a non-metal of group VI of the periodic table; Y is a member of the sulfur family; x is an integer from 1 to 4; and R' is an organic group which may be either aryl, alkyl, aralkyl, or alkyl-aryl, and which may contain substituent atoms or groups, such as halogen, nitro, amino, hydroxy, alkoxy, aroxy, mercapto, carboxy, and the like. The metals which may be substituted for the hydrogen in the  $-\text{XH}$  group of the above formula in forming salts of such compounds may be any metals, the most important for the purposes of the present invention being calcium, barium, strontium, magnesium, and zinc, although for some purposes corresponding compounds containing tin, lead, aluminum, cobalt or nickel will also be found to be especially desirable.

Compounds particularly suited for the purposes of the present invention are formed by reacting sulfur with a compound of the formula



where R represents at least one alkyl radical attached to the nucleus, the total number of carbon atoms in all of such radicals being at least five when the compound is to be dissolved in hydrocarbon oils, X is oxygen or sulfur, M is a divalent metal of group II of the periodic table, and x is an integer from 1 to 4.

It should be understood that the above general formulas include compounds in which various

## 4

substituent atoms or groups may be attached to the aromatic nucleus, such as alkyl, cycloalkyl, aralkyl, aryl, carboxyl, hydroxyl, alkoxy, aroxy, sulphydryl, nitro, ester (organic and/or inorganic), keto, amino, aldehydo, chloromethyl, aminomethyl, alkyl thiomethyl, alkyl xanthomethyl, metal substituted carboxyl, metal substituted sulfonic acid, metal substituted hydroxyl or sulphydryl groups, halogen atoms, etc. Different types of atoms or groups may be attached to the same aromatic nucleus. Alkyl radicals attached to the nucleus may have a total of five to twelve carbon atoms in all of such groups, but in some cases as many as sixteen to twenty or more carbon atoms in a single group, or a plurality of groups, may be preferred. If more than one alkyl group is present in a single molecule, whether or not attached to the same aryl nucleus, such groups may be alike or different. Such alkyl or other hydrocarbon groups may contain substituent groups, such as those named above as substituents in the aromatic nucleus. The positions of the various groups or atoms attached to the aromatic nucleus may be any positions relative to one another.

Alkyl phenol sulfides, whose metal salts may be used to prepare the reaction products of the present invention, may be illustrated by the following general classes of compounds:

1. Alkyl phenol thioethers:



2. Alkyl phenol disulfides:



and



3. Polymers of alkyl phenol sulfides:



In all of the above formulas under the headings 1 to 3 R represents at least one alkyl group containing preferably at least four carbon atoms, m is a small whole number not greater than about six, and x is a small whole number from 1 to 4.

When the products are to be employed as addi-

4,09,687

2,409,687

5

5  
tives for lubricating oils, exceptionally good results can be obtained by employing metal salts of alkyl phenol sulfides having C<sub>16</sub>—C<sub>20</sub> branched chain alkyl groups. These can be conveniently prepared from phenols which have been alkylated with what are essentially branched chain polymers of n-butene obtained as by-products in the manufacture of secondary butyl alcohol from petroleum refinery C<sub>4</sub> hydrocarbon fractions.

It should be understood that generally, throughout this specification, the term "alkyl phenol sulfide" is meant to include not only the monosulfides but also the di- and polysulfides and polymers of alkyl phenol sulfides as well. Thus, although reaction of an alkylated phenol with sulfur dichloride (S<sub>2</sub>Cl<sub>2</sub>) will give essentially an alkyl phenol monosulfide, small amounts of polysulfides and of polymeric materials will also be formed. This is even more usually the result when more than the theoretically required proportion of sulfur halide is used in preparing the alkyl phenol sulfide, as, for example, when 2 moles of alkyl phenol sulfide are treated with 1.5 moles of sulfur dichloride. Similarly, the alkyl phenols may be treated with more than theoretical quantities of sulfur monochloride (S<sub>2</sub>Cl<sub>2</sub>) or with mixtures of sulfur mono- and dichloride or with first one halide and then the other.

Other compounds whose metal salts may be used in accordance with this invention are illustrated by the following:



In these formulas R, R', etc., represent organic 70 radicals, preferably alkyl groups.

In all of the above described type formulas, both general and specific, where R is used to represent an organic radical, such radicals may be illustrated by the following species, which are 75

6

radicals particularly preferred in the compounds, it being understood that the list is merely illustrative and does not restrict the scope of the groups of the formulas. These include n-butyl, 5 isobutyl, tert.-butyl, n-amyl, isoamyl, cyclohexyl, n-octyl, isoctyl, tert.-octyl, dodecyl, octadecyl, wax chain and C<sub>16</sub>—C<sub>24</sub> branched chain radicals.

Structures of several typical compounds whose salts may be reacted with sulfur in accordance 10 with the present invention may be given to show what is believed to be the relative positions of the various groups in the aromatic nuclei, but it is to be understood again that these formulas are given as illustrations only. These typical examples are the following:

(a)



(b)



(c)



(d)



40 Specific examples of compounds which may be treated with sulfur in accordance with the present invention include the following, which are not to be construed as limiting the invention in any manner:

45 Calcium tert.-octyl phenol sulfide

Barium 2,4-di-tert.-amyl phenol sulfide

Cobalt tert.-amyl phenol sulfide

50 Barium salt of 2-hydroxy-3,5-di-tert.-amyl-4'-diethylamino diphenyl sulfide

Zinc salt of salicylic acid sulfide octyl ester

Barium 2-stearoyl-4-amyl phenol sulfide

Mixed calcium-barium tert.-octyl phenol sulfide

55 Tin salt of C<sub>16</sub>—C<sub>20</sub> branched chain alkyl phenol sulfide

Barium salt of bis(2,4-diamyl phenol)-4-amylphenol dithioether (prepared from 2 moles of 2,4-di-tert.-amyl phenol and one mole of p-tert.-amyl phenol, sulfurized with sulfur chloride and neutralized with barium hydroxide)

60 When the salts employed are those of polyvalent metals, it is not essential that all of the valences be satisfied by hydroxyaryl sulfide groups; some of them may be satisfied by other acidic organic groups such as carboxy, aroxy, alkoxy, organo-substituted inorganic acid groups such as phosphoric, phosphorous, thiophosphoric, thiophosphorous, sulfonic, sulfinic, phosphonic, phosphinic, and the like.

Thus, for example, the present invention also includes reaction products of sulfur with such compounds as:

Calcium mixed salt of tert.-amyl phenol sulfide and iso-octyl salicylate

- Aluminum mixed salt of tert.-octyl phenol sulfide and stearic acid  
 Tin mixed salt of di-tert.-amyl phenol sulfide and naphthenic acids  
 Barium mixed salt of tert.-octyl phenol sulfide and petroleum mahogany sulfonic acids 5  
 Nickel mixed salt of tert.-amyl phenol sulfide and amyl xanthic acid  
 Zinc mixed salt of isododecyl phenol sulfide and methyl cyclohexyl thiophosphoric acid  
 Nickel mixed salt of tert.-amyl phenol sulfide and oleic acid  
 Magnesium mixed salt of tert.-octyl phenol sulfide and cetyl phenol

As has been mentioned previously in this specification, the term phenol sulfide is meant to include not only the monosulfide but also disulfides, polysulfides, or polymers or mixtures of any of these in any proportion.

For the objects stated, the metal salts of alkylated phenol sulfides have been preferably prepared from phenolic compounds readily obtained by synthetic alkylation of the simple phenols, followed by treatment with a sulfur chloride, and then neutralization with a metallic base.

Suitable synthetic alkyl phenols for preparing the desired phenol sulfide salts are preferably those containing secondary or tertiary alkyl radicals because alkylation of a simple phenol occurs more readily with branched aliphatic reactants. Commonly, the alkylation reaction involves a condensation of olefins with the simple phenols, the reaction being catalyzed by anhydrous metal halides, boron fluoride, hydrofluoric acid, 35 stannic chloride with hydrogen chloride, sulfuric acid, phosphoric acid or certain activated clays. As olefinic reactants, refinery gases containing propylene, butylenes, amylenes, etc., are economically useful, although individual olefins or olefin-containing mixtures derived from other sources may be used. Preferred individual olefins are the butenes, amylenes, and olefin polymers, such as diisobutylene or triisobutylene, or normal olefin polymers or copolymers of normal 45 and secondary or tertiary olefins, or copolymers of olefins and diolefins. The reaction temperature is usually controlled to avoid side reactions. In employing sulfuric acid, a liquid phase reaction at relatively low temperature is preferred, while with phosphoric acid the reaction may be carried out in the vapor phase.

Suitable alkylated phenols for conversion to phenol sulfides may be thus prepared by alkylating phenol, cresol, naphthol or other phenolic compounds. High molecular weight alkylated phenols may also be used, for example, those prepared by condensing phenols with chlorinated petrodatum or chlorinated paraffin wax or with a chlorinated kerosene or gas oil. Naturally occurring phenols, such as those obtained by alkaline extraction of certain petroleum stocks or those obtained from cashew nut shell liquid or those obtained from other vegetable oil sources may likewise be used. Halogenated or nitrated 55 phenols will also find application in this invention, particularly if the final additive is to be employed in extreme pressure lubricants.

One class of alkyl phenols which are particularly preferred are those which have been prepared by alkylation of phenol with an olefin polymer such as diisobutylene or a refinery butene polymer oil. Alkylation of phenol with about an equal molar proportion of diisobutylene gives p-tert.-octyl phenol, also known as diisobutyl phe-

nol or tetramethyl butyl phenol. This phenolic material is especially desirable because of the ease of its preparation and because products made from it are highly satisfactory for the present invention. In many instances, however, a higher degree of alkylation may be advantageous, and for this reason the phenol may be alkylated with as much as two molecular equivalents of diisobutylene to give, under proper conditions, 10 essentially di-tert.-octyl phenol; or it may be alkylated with other olefin polymers such as triisobutylene, or other isobutylene polymers. For many purposes it is preferable to employ alkylated phenols having branched chain alkyl groups of from 16 to 30 carbon atoms. Suitable products may be prepared by alkylating phenol with certain of the polymeric materials obtained as by-products in the manufacture of butyl alcohol from petroleum refinery butenes. 15 These consist essentially of polymers of n-butene with small percentages of isobutene and other olefins and give alkylated phenols having branched chain alkyl groups of 16-29 or 20-24 carbon atoms, depending on the polymeric material used in the alkylation. It should be understood that in many cases the alkylation products may be mixtures of various compounds rather than entirely one specific alkyl phenol, and that it is intended to use such mixtures in practicing this invention.

For conversion of phenols to phenol sulfides the phenol is reacted with sulfur dichloride to produce essentially a phenol monosulfide having a thioether linkage, while sulfur monochloride may be used to produce essentially the phenol disulfide. About one-half to one mol of sulfur halide is used with each mol of phenol, and the reaction is preferably carried out in a solvent such as dichlorethane, choloform, petroleum naphtha, benzol, xylol, toluol, and the like.

For converting the phenol sulfides to metal salts, it is usually sufficient merely to add a metal or a metallic oxide, hydroxide, sulfide, alkoxide, hydride, or carbide to a mineral oil solution or other solution of the phenol sulfide at an elevated temperature. Thus, barium salts of alkylated phenol sulfides are prepared by reacting the sulfide with barium hydroxide, preferably in the form of the hydrate,  $Ba(OH)_2 \cdot 8H_2O$ . The calcium salts may be prepared by reacting alkyl phenol sulfides with calcium methylate or other calcium alcoholate. In some instances it may be preferable to prepare heavy metal salts from the alkali metal salt by double decomposition. 55 In many cases the metal alkyl phenol sulfide prepared by neutralization with a metal hydroxide may occur as a hydrated salt. Use of hydrated salts prepared in this manner or by any other method is also contemplated in the processes of the present invention.

In accordance with the present invention, the metallic salt of a phenol sulfide or other metallic derivative of a hydroxy or mercapto aromatic sulfide is caused to react with sulfur. This may be accomplished by adding the sulfur in elemental form to a heated solution of the metallic compound. The sulfur may be used in any of its allotropic forms.

In carrying out the reaction described above the proportions of sulfur and metal salt of phenol sulfide are so chosen that from 0.1 to 2.5 atomic proportions of sulfur are reacted with one atomic proportion of metal, the preferred ratio being within the limits of about 0.5 to 1.5 atomic proportions of sulfur for each atomic pro-

100

2,409,687

9

portion of metal. This preferred ratio gives the products the optimum content of sulfur to impart to them the maximum amount of inhibiting power.

If desired, the products used in accordance with this invention may be prepared by the simultaneous reaction of a phenol sulfide, a metal oxide or hydroxide and elemental sulfur. However, in order to avoid the formation of oil-insoluble materials, it is preferred to first form the metal salt of the phenol sulfide and then react this with sulfur.

Although the reaction can be brought about by fusing the metal salt with sulfur, it is more convenient to carry out the reaction with the aid of solvents, particularly high boiling hydrocarbon solvents, such as xylol or a petroleum fraction. A particularly preferred reaction medium is a lubricating oil fraction, since the final reaction product can thus be obtained as a mineral oil concentrate of the desired additive, which may be conveniently shipped or stored as such and then readily blended with the lubricating oil base stock in the desired concentration to form a finished lubricating oil blend.

The additives may generally be prepared by first dissolving an alkylated phenol sulfide in a mineral oil or other suitable solvent and treating the same with a metal hydroxide, e. g.,



at about 80-200° C., preferably 110°-150° C. After a further period of heating free sulfur is added, heating being continued at 100-230° C., preferably at 150-200° C., to complete the reaction. The period of heating will generally be from about 10 minutes to 1 hour, although in some cases a longer period may be required. When the material will no longer stain a strip of copper immersed in it for about 10 seconds at 180-190° C., the reaction is considered complete. The product is then filtered, giving a concentrate of the desired additive. If the products are found to have a slight odor of hydrogen sulfide, this can be substantially eliminated by treating with a small proportion (2-5%) of barium hydroxide or calcium oxide or hydroxide at 150° C., followed by filtering and blowing with nitrogen at 100°-120° C. In some cases improved products may be obtained by heat treatment of the metal phenol sulfide before or after reaction with sulfur. The heat treatment may be conducted, for example, at 150° C. for 10-15 hours.

It has been found that good results are obtained when preparing these additives in mineral oil if a minor proportion of a higher alcohol, such as stearyl, lauryl or cetyl alcohol, or wool fat alcohol or the like, is added to the reaction mixture in which the compounds of the present invention are prepared. This alcohol reduces foaming during the process and acts as an auxiliary solvent for the final product. The best results are obtained by adding a sufficient quantity of alcohol to give a concentration of about 3% to about 15% in the final additive concentrate. It has been determined by test that substantially none of the higher alcohol enters into the reaction.

It has also been found that products of better oil solubility can often be obtained when carrying out the reaction with sulfur in the presence of a small proportion of an olefinic material, such as a tetraisobutylene, cracked wax or an unsaturated alcohol.

Generally, the additives of the present invention are most advantageously blended with lubri-

10

cating oil base stocks in concentrations between the approximate limits of 0.02% and 5.0% and preferably from 0.1% to 2.0%, although larger amounts may be used for some purposes. The

exact amount of addition agent required for maximum improvement depends to a certain extent on the particular products used, the nature of the lubricating oil base stock and the general operating conditions of the engine in which the lubricant is to be employed. This same general range of concentration will also be effective when the additives are to be used in greases and in extreme pressure lubricants, although in the latter instance greater amounts, up to 20%, may also be employed.

It has been pointed out elsewhere in this specification, it is often convenient to prepare concentrates of the additives in oil, containing, say, 25 to 75% of effective addition agent, the concentrate later being added to a suitable lubricating oil base stock to give a finished blend containing the desired percentage of additive. Thus, when using a 40% concentrate, 2.5% of this material may be blended with a suitable base stock to give a finished oil containing 1% of effective addition agent.

In the following examples are described various preparations of products in accordance with this invention and the results obtained on testing the same in various lubricating oil blends. It is to be understood that these examples, given for illustrative purposes only, are not to be construed as limiting the scope of the invention in any way.

#### Example 1

35 Tertiary octyl phenol was prepared by alkylating phenol with diisobutylene, using stannic chloride and HCl catalysts substantially as described in the Buc U. S. Patent 2,332,555.

40 A 30% solution of tert.-octyl phenol was prepared by dissolving 100 parts by weight of the alkylated phenol in 233 parts of chloroform. Then over a period of three hours 37.5 parts of sulfur dichloride was added, the temperature being maintained at 20-25° C. Agitation was continued for an additional hour at the same temperature, after which the solution was heated under reflux for two hours. The solvent was stripped off at a maximum temperature of 100° C. and the 45 alkyl phenol sulfide blown with carbon dioxide until free of HCl. The resulting tert.-octyl phenol sulfide was a dark brown resinous product completely soluble in mineral oils.

382 parts by weight of solvent-free tert.-octyl

55 phenol sulfide prepared as above was dissolved in 618 parts of refined mineral lubricating oil (52 seconds Saybolt viscosity at 210° F.) at a temperature of 70-80° C. To the agitated oil solution 125 parts of commercial stearyl alcohol was added and the temperature was then raised to

60 105-110° C. Then 278 parts of barium hydroxide octahydrate,  $\text{Ba(OH)}_{2.8}\text{H}_2\text{O}$ , was gradually added in small portions, the rate of addition being governed by the amount of foaming of the reaction mixture. During this step the mixture was blown with nitrogen to facilitate removal of water vapor. Following the addition of the barium hydroxide, agitation and blowing were continued at

65 110° C. for 30 minutes, then Hyflo filter aid was added (2 lbs. per 100 gallons of mixture), the temperature raised to 125° C. and the mixture filtered through a filter press, the concentrate being recycled until a perfectly clear product was obtained. The final product was a mineral oil 70 concentrate containing 40% barium tert.-octyl

75

## 11

phenol sulfide, 10% stearyl alcohol, and 50% mineral lubricating oil. It contained 3.2% sulfur and 9.3% barium.

## Example 2

As starting material for the preparation of a reaction product of a barium salt, there was used a concentrate containing 40% by weight of barium tert.-octyl phenol sulfide, 10% of stearyl alcohol and 50% of a refined mineral oil of 52 seconds viscosity Saybolt at 210° F., prepared as described in Example 1. 500 g. of this concentrate was treated with 10 g. of sulfur by heating the concentrate to 120° C. and adding the sulfur gradually with agitation over a period of 10 minutes, during which the temperature rose to 190° C. The temperature was then held at 160°-180° C. for a total reaction period of 2½ hours and the final product filtered. The resulting material contained 4.87% sulfur.

## Example 3

The purpose of the following test was to determine the corrosion inhibiting effect of adding a small quantity of the product prepared as in the preceding example to a lubricating oil base, this being a well refined solvent extracted paraffinic type mineral lubricating oil of S. A. E. 20 grade. The oil contained 0.625% of additive concentrate prepared in accordance with Example 2, which is equivalent to about 0.25% of the actual additive. A comparative test was made with a sample of the unblended oil base.

The tests were conducted as follows: 500 cc. of oil to be tested was placed in a glass oxidation tube (13" long and 2½" diameter) fitted at the bottom with a ¼" bore air inlet tube perforated to facilitate air distribution. The oxidation tube was then immersed in a heated bath so that the oil temperature was maintained at 325° F. during the test. Two quarter sections of automotive bearings of copper-lead alloy of known weight having a total area of 25 sq. cm. were attached to opposite sides of a stainless steel rod which was then immersed in the oil and rotated at 600 R. P. M., thus providing sufficient agitation of the sample during the test. Air was then blown through the oil at the rate of 2 cu. ft. per hour. To increase the severity of the test, the bearings were washed and weighed at the end of each four hour period and then polished and reweighed before continuing for another four hour period. The results, given in Table I, show the cumulative weight loss at the end of each four hour period.

Table I

| Oil blend                               | Cumulative bearing weight loss<br>(mg./25 sq. cm.) |        |         |         |         |         |
|-----------------------------------------|----------------------------------------------------|--------|---------|---------|---------|---------|
|                                         | 4 hrs.                                             | 8 hrs. | 12 hrs. | 16 hrs. | 20 hrs. | 24 hrs. |
| Base oil                                | 0                                                  | 173    | —       | —       | —       | —       |
| Base oil+0.625% product of<br>Example 2 | 0                                                  | 0      | 10      | 31      | 94      | 297     |

Although in most instances the additives of the present invention will of themselves impart sufficient improvement to lubricating oils to give very satisfactory results, still greater improvement may often be obtained by employing these addition agents in conjunction with other additives of the detergent type, such as metal soaps, metal phenates, metal alcoholates, metal phenol sulfides, metal organo phosphates, thiophos-

## 12

phates, phosphites and thiophosphites, metal sulfonates, metal thiocarbamates, metal xanthates and thioxanthates, and the like.

Thus the addition agents of our invention may be used in mineral lubricating oils in conjunction with one or more of the following representative materials:

|     |                                                                                  |
|-----|----------------------------------------------------------------------------------|
| 10  | Barium tert.-octyl phenol sulfide                                                |
| 15  | Barium di-tert.-amyl phenol sulfide                                              |
| 20  | Cobalt tert.-amyl phenol sulfide                                                 |
| 25  | Tin salt of wax alkylated phenol sulfide                                         |
| 30  | Calcium mahogany sulfonates                                                      |
| 35  | Barium mahogany sulfonates                                                       |
| 40  | Strontium mahogany sulfonates                                                    |
| 45  | Magnesium mahogany sulfonates                                                    |
| 50  | Calcium isohexadecyl phenol sulfonate                                            |
| 55  | Calcium double salt of octadecyl phenol sulfonic acid                            |
| 60  | Barium phenate-zinc sulfonate of isohexadecyl phenol sulfonic acid               |
| 65  | Calcium salt of amyl phenol-formaldehyde condensation product                    |
| 70  | Magnesium cetyl phenate                                                          |
| 75  | Calcium ortho stearoyl phenate                                                   |
| 80  | Nickel oleate                                                                    |
| 85  | Calcium dichlorostearate                                                         |
| 90  | Calcium phenyl stearate                                                          |
| 95  | Barium octadecylate                                                              |
| 100 | Aluminum-calcium mixed soap of fatty acids from oxidation of petroleum fractions |
| 105 | Nickel dibutyl dithiocarbamate                                                   |
| 110 | Nickel amyl xanthate                                                             |
| 115 | Barium dioctyl dithiophosphate                                                   |
| 120 | Zinc methyl cyclohexyl dithiophosphate                                           |
| 125 | Calcium dihexadecyl monothiophosphate                                            |
| 130 | Zinc tert.-octyl phenol sulfide thiophosphate                                    |
| 135 | Calcium cetyl phosphate                                                          |
| 140 | Magnesium lauryl salicylate                                                      |
| 145 | Zinc diisopropyl salicylate                                                      |
| 150 | Calcium phenate-barium carboxylate of octadecyl salicylic acid                   |
| 155 | Tin naphthenate                                                                  |
| 160 | Aluminum naphthenate                                                             |

Particularly advantageous are lubricant compositions in which the additives of the present invention are employed in conjunction with metal salts of petroleum mahogany sulfonic acids. Examples of such compositions include the following:

|                                                                                                     | Per cent |
|-----------------------------------------------------------------------------------------------------|----------|
| 1. Additive concentrate containing 40% of sulfur-barium tert.-octyl phenol sulfide reaction product | 1.0      |
| 55 Calcium mahogany sulfonates                                                                      | 1.5      |
| 55 Mineral lubricating oil                                                                          | 97.9     |
| 2. Additive concentrate containing 35% of sulfur-calcium tert.-amyl phenol sulfide reaction product | 2.5      |
| 60 Barium mahogany sulfonates                                                                       | 1.5      |
| 60 Mineral lubricating oil                                                                          | 96       |
| 3. Zinc mahogany sulfonates                                                                         | 2.3      |
| 65 Additive concentrate containing 40% of sulfur-barium-2,4-diamyl phenol sulfide reaction product  | 2.0      |
| 65 Mineral lubricating oil                                                                          | 94       |

The lubricating oil base stocks used in the compositions of this invention may be straight mineral lubricating oils or distillates derived from paraffinic, naphthenic, asphaltic or mixed base crudes, or, if desired, various blended oils may be employed as well as residuals, particularly those from which asphaltic constituents have been carefully removed. The oils may be refined by

## 13

conventional methods using acid, alkali and/or clay or other agents such as aluminum chloride, or they may be extracted oils produced, for example, by solvent extraction with solvents of the type of phenol, sulfur dioxide, furfural, dichloro ethyl ether, nitrobenzene, crotonaldehyde, etc. Hydrogenated oils or white oils may be employed as well as synthetic oils prepared, for example, by the polymerization of olefins or by the reaction of oxides of carbon with hydrogen or by the hydrogenation of coal or its products. In certain instances cracking coil tar fractions and coal tar or shale oil distillates may also be used. Also, for special applications, animal, vegetable or fish oils or their hydrogenated or volatilized products may be employed, either alone or in admixture with mineral oils.

For the best results the base stock chosen should normally be that oil which without the new additives present gives the optimum performance in the service contemplated. However, since one advantage of the additives is that their use also makes feasible the employment of less satisfactory mineral oils or other oils, no strict rule can be laid down for the choice of the base stock. Certain essentials must of course be observed. The oil must possess the viscosity and volatility characteristics known to be required for the service contemplated. The oil must be a satisfactory solvent for the additive, although in some cases auxiliary solvent agents may be used. The lubricating oils, however they may have been produced, may vary considerably in viscosity and other properties depending upon the particular use for which they are desired, but they usually range from about 40 to 150 seconds Saybolt viscosity at 210° F. For the lubrication of certain low and medium speed Diesel engines the general practice has often been to use a lubricating oil base stock prepared from naphthenic or aromatic crudes and having a Saybolt viscosity at 210° F. of 45 to 90 seconds and a viscosity index of 0 to 50. However, in certain types of Diesel service, particularly with high speed Diesel engines, and in aviation engine and other gasoline engine service, oils of higher viscosity index are often preferred, for example, up to 75 to 100, or even higher, viscosity index.

In addition to the materials to be added according to the present invention, other agents may also be used, such as dyes, pour depressors, heat thickened fatty oils, sulfurized fatty oils, organo metallic compounds, metallic or other soaps, sludge dispersers, antioxidants, thickeners, viscosity index improvers, oiliness agents, resins, rubber, olefin polymers, volatilized fats or fatty oils, volatilized mineral oils, and/or volatilized waxes and colloidal solids such as graphite or zinc oxide, etc. Specific examples of such other agents include phenyl alpha-naphthylamine, volatilized sperm oil, 2,6-di-tert.-butyl-4-methyl phenol, sulfurized sperm oil, p-tert.-amyl phenol sulfide, dibenzyl disulfide, polyisobutylene, sulfurized wax olefins, tricresyl phosphate, diamyl trisulfide, and the condensation product of phenol with a sulfur chloride-diisobutylene reaction product. Solvents and assisting agents, such as esters, ketones, alcohols, amines, nitriles, aldehydes, halogenated or nitrated compounds, and the like, may also be employed.

Assisting agents which are particularly desirable are the higher alcohols having eight or more carbon atoms and preferably 12 to 20 carbon atoms. The alcohols may be saturated straight and branched chain aliphatic alcohols such

## 14

as octyl alcohol ( $C_8H_{17}OH$ ), lauryl alcohol ( $C_{12}H_{25}OH$ ), cetyl alcohol ( $C_{16}H_{33}OH$ ), stearyl alcohol, sometimes referred to as octadecyl alcohol ( $C_{18}H_{37}OH$ ), heptadecyl alcohol ( $C_{17}H_{35}OH$ ), and the like; the corresponding olefinic alcohols, such as oleyl alcohol; cyclic alcohols, such as naphthenic alcohols; and aryl substituted alkyl alcohols, for instance, phenyl octyl alcohol, or octadecyl benzyl alcohol or mixtures of these various alcohols, which may be pure or substantially pure synthetic alcohols. One may also use mixed naturally occurring alcohols such as those found in wool fat (which is known to contain a substantial percentage of alcohols having about 16 to 18 carbon atoms) and in sperm oil (which contains a high percentage of cetyl alcohol); and although it is preferable to isolate the alcohols from those materials, for some purposes, the wool fat, sperm oil or other natural products rich in alcohols may be used per se. Products prepared synthetically by chemical processes may also be used such as alcohols prepared by the oxidation of petroleum hydrocarbons, e. g., paraffin wax, petrolatum, etc.

These assisting agents serve to enhance the detergent and sludge dispersive qualities and aid the solubility of the metal-containing additives and at the same time impart some oiliness properties to the lubricating oil compositions.

In addition to being employed in crankcase lubricants, the additives of the present invention may also be used in extreme pressure lubricants, engine flushing oils, industrial oils, heat transfer media, general machinery oils, steam cylinder oils, cutting oils, insulating oils, process oils, rust preventive compositions, hydraulic oils and greases. Also their use in motor fuels, Diesel fuels and kerosene is contemplated. A particular application in this regard is their use in motor fuels containing tetraethyl lead or other anti-knock agents, the additives of the present invention serving not only as antioxidants for the fuel but also as stabilizers for the anti-knock agent itself. Since these additives exhibit antioxidant properties and are believed also to possess ability to modify surface activity, they may be employed in asphalts, road oils, waxes, fatty oils of animal or vegetable origin, soaps and plastics. Similarly, they may be used in natural and synthetic rubber compounding both as vulcanization assistants and as antioxidants, and generally they may be used in any organic materials subject to deterioration by atmospheric oxygen.

The present invention is not to be considered as limited by any of the examples described herein which are given by way of illustration only, but it is to be limited solely by the terms of the appended claims.

We claim:

1. As a new composition of matter an oil-soluble sulfur containing product obtained by reacting elemental sulfur with a compound of the formula



70 where R is an alkyl radical of at least 5 carbon atoms, X is a member of the group consisting of oxygen and sulfur, M is a divalent metal of group II of the periodic table and selected from the 75 group consisting of calcium, barium, strontium,

15

magnesium, and zinc, and  $x$  is an integer from 1 to 4.

2. The method of preparing an oil-soluble sulfur containing product having antioxidant properties in the presence of organic materials which comprises reacting elemental sulfur with a compound of the formula



where R is an alkyl radical of at least 5 carbon atoms, X is a member of the group consisting of oxygen and sulfur, M is a divalent metal of group II of the periodic table and selected from the group consisting of calcium, barium, strontium, magnesium, and zinc, and  $x$  is an integer from 1 to 4.

16

DILWORTH T. ROGERS.  
JOHN G. McNAB.

10